

# UNITED STATES PATENT OFFICE.

JOHN H. YOCUM, OF EAST ORANGE, NEW JERSEY, ASSIGNOR TO THE CLARENDON-YOCUM COMPANY, OF NEWARK, NEW JERSEY, A CORPORATION OF NEW JERSEY.

## PROCESS FOR TREATING HIDES.

1,175,495.

Specification of Letters Patent. Patented Mar. 14, 1916.

No Drawing. Original application filed April 17, 1913, Serial No. 761,748. Divided and this application filed June 18, 1915. Serial No. 34,815.

*To all whom it may concern:*

Be it known that I, JOHN H. YOCUM, a citizen of the United States, and resident of East Orange, in the county of Essex and 5 State of New Jersey, have invented certain new and useful Improvements in Processes for Treating Hides, of which the following is a specification.

My invention relates to a process for treating 10 fresh or green hides to preserve them for tanning purposes, and it has for its object to prevent the discoloration which occurs during the tanning process with hides preserved by present methods. These discolorations, commonly called salt stains, 15 prevent the use of the leather in light colors, such as the tans, and require that the leather be artificially colored to cover up the stains.

20 By my invention the fresh hides are treated with a compound composed of common salt and a small proportion of the normal sulfite of sodium, or the normal sulfite of a similar base, such as potassium, ammonium, 25 etc. This composition consists preferably of about 97 per cent. of common salt (sodium chlorid) and about 3 per cent. of normal sulfite of sodium. The percentage of the sulfite may be increased as high as 6 per 30 cent. and as low as 2 per cent., but I have found that the above preferred proportions give the best results for the average run of 35 hides.

Usually the fresh hides are obtained in 40 quantities at packing houses or slaughter houses, and in applying my process the hides or skins are laid one on top of the other with the hair side down. As each hide is 45 covered with a composition powder. These bundles of treated hides are preserved in this condition until they are ready to be shipped to the tanner.

In making up the composition, the ingredients in the proper proportion are thoroughly mixed so that the sulfite is evenly distributed throughout the mixture.

While I have mentioned only common salt, or sodium chlorid, as the main in-

50 gredient in the compound, and while I prefer to use sodium chlorid, other neutral salts of sodium, such as sodium sulfate, may be substituted in place of the chlorid.

By the use of my process the discoloration 55 of preserved hides during the subsequent tanning treatment, and the formation of salt stains, is entirely prevented. Hides or skins which have been preserved by my process are of a uniform color when properly tanned.

Having thus described my invention, what I claim is:

1. In the process of preserving fresh hides for tanning purposes, the step which consists in partially covering the hides with a 65 composition containing sodium chlorid and a small percentage of a normal sulfite of an alkali metal.

2. In the process of preserving fresh hides for tanning purposes, the step which consists in partially covering the hides with a 70 composition containing sodium chlorid and a small percentage of normal sulfite of sodium.

3. In the process of preserving fresh hides 75 for tanning purposes, the step which consists in partially covering the hides with a composition containing approximately 97 per cent. of sodium chlorid and approximately 3 per cent. of a normal sulfite of an 80 alkali metal.

4. In the process of preserving fresh hides for tanning purposes, the step which consists in partially covering the hides with a 85 composition containing approximately 97 per cent. of sodium chlorid and approximately 3 per cent. of normal sulfite of sodium.

5. In the process of preserving fresh hides 90 for tanning purposes, the step which consists in partially covering the hides with a composition containing common salt intimately associated with approximately 3 per cent. of normal sulfite of sodium.

Signed at New York, in the county of 95 New York, and State of New York, this 16th day of June, A. D. 1915.

JOHN H. YOCUM.